

Oct. 11, 1932.

H. W. SERVER

1,882,194

PROCESS OF PAPER MANUFACTURE

Filed Jan. 22, 1930



INVENTOR  
HERBERT W. SERVER.

BY *Taubman & Taubman*  
ATTORNEYS

## UNITED STATES PATENT OFFICE

HERBERT W. SERVER, OF DAYTON, OHIO

## PROCESS OF PAPER MANUFACTURE

Application filed January 22, 1930. Serial No. 422,502.

My invention relates to a process of paper manufacture.

It is a particular object of my process to manufacture paper which is made from waste paper in order to reduce the introduction of costly paper stocks, to give greater strength to the resulting product and to form a product from which water flows more easily in the machine, thereby increasing the rate of production of the paper.

It is a further object to provide a paper of better printing quality as well as of greater strength.

It is an especial object of my invention to provide a paper through my new process in which a material saving in cost in bleaching materials, such as bleaching chlorine, will be effected.

It is an object to provide a process in which it is possible to omit bleached sulphite entirely.

It is an object to get a brighter and better color to the finished sheet of paper.

Referring to the drawing:

Figure 1 is a diagrammatic perspective of the apparatus which may be employed as a typical installation for the practice of my process, but it will be understood that other forms and arrangements of apparatus may be employed;

Figure 2 is a vertical section through two of the several bleaching towers.

Referring to the drawing in detail, it is a feature of my process to introduce unbleached sulphite or unbleached sulphate at any place in the process of manufacture of paper from the primary beater to the exit of the stock from the rotary screens prior to entry into the bleaching towers or into the stream entering the bleaching towers.

I have shown in Figure 1 a preferred form of introducing the raw sulphite or raw sulphate in its unbleached condition but do not desire to be confined to that arrangement.

Referring to the drawing in detail, 1 is a beater in which is introduced paper stock, such as magazine stock. Heretofore, it has been the practice to also introduce the more expensive ledger stock in order to give strength and superior printing surface to

the resulting product. In the present process, it is possible to eliminate ledger stock entirely. In the previous process, difficulty has always been found in the manufacture of paper from such stock that the fibers were so fine or short, or both, that they made a very dense paper stock from which the water would not flow readily and, therefore, necessitated a relatively slow production. The length of the fibers in such paper was relatively short and, therefore, the paper was relatively weak.

It is now the practice to put unbleached sulphite in the beaters subsequent to the bleaching towers.

Referring again to Figure 1, the magazine stock or its equivalent proceeds from the beater through the system of pipes designated 2 to the cooker tanks 3 which are supplied with steam through the pipes 4. In these tanks the steam at 190 degrees bubbles up through the tanks breaking up the stock and de-inking it.

The resultant product passes through the pipes 5 into the storage tank 6. It is withdrawn from that tank through the pipe 7 by the pump 8 which, at the same time, draws surplus return liquor through the pipe 9 from the rotary screens hereinafter described. This joint product is discharged by the pump 8 through the pipe 10 into the tank 11 whence it passes through the pipes 12 through the riffle tanks 13 which settle out the foreign material. It then proceeds to the piping system 14 into screen tanks 15 having screens 16 whence it makes its exit from the stock box line 17 into the first rotary screen box 18 from which the waste liquor goes to waste through the pipe 19. The resulting product enters the successive screen boxes through piping means not shown, or equivalent means, to the boxes 20, 21 and 22 containing suitable rotary screens. The liquor from the boxes is transported, as indicated by the arrows, through the pipes 23, pump 24, pipe 25, pipe 26, pump 27, pipe 28 and pipe 9. Bleaching chlorine is introduced through the pipe 29 into the product in the sump 31. The product passes through the pipe 30 into a sump 31. Raw sulphite is beaten in the beater 32

and passes through the pipe 33 into the sump 31. The joint product then passes from the pipe 34 into the first bleaching tower 35 which is provided with stirrers 36. The stock flows from tower to tower, such as towers 37, 38, 39, 40 and 41 by pipes designated 42 and thence out to the paper machine by the pipe 43.

10 It will be understood that the raw sulphite can be introduced into the system anywhere through the course of manufacture of the paper stock.

It will also be understood that raw sulphite and raw sulphate are used interchangeably.

15 It will be understood that I desire to comprehend within my invention such modifications as may be necessary to adapt it to varying conditions and uses. It will be further understood that when I say unbleached sulphite I include partly bleached sulphite.

Having thus fully described my invention, what I claim as new and desire to secure by Letters Patent, is:—

20 1. In a process of making paper, disintegrating the stock, introducing raw sulphite therein and bleaching the stock by adding bleach and passing the stock through a succession of bleaching towers.

25 2. In a process of making paper, disintegrating the stock, introducing raw sulphite therein, bleaching the stock by chlorine bleach and passing the stock through a succession of bleaching towers.

30 3. In a process of making paper, beating refuse paper stock, de-inking said stock, introducing bleach into said stock, introducing raw sulphite into said stock and passing the stock through a succession of bleaching towers.

35 4. In a process of manufacturing paper from refuse stock, beating the refuse stock, cooking it, screening it, introducing bleach into it, introducing raw sulphite into it and passing the stock through a succession of

40 bleaching towers.

45 5. In a process of manufacturing paper from refuse stock, beating the refuse stock, cooking it, introducing bleach into it, introducing raw sulphite into it and passing the stock through a succession of bleaching towers.

50 6. In a process of manufacturing paper from refuse paper stock having relatively short fibers, beating the stock, screening the stock, introducing raw sulphite into the stock and passing the stock through a succession of bleaching towers.

55 7. In a process of manufacturing paper from refuse paper stock having relatively short fibers, beating the stock, screening the stock and introducing raw sulphite into the stock, and introducing bleach into the stock.

60 8. In a process of manufacturing paper from refuse paper stock having relatively short fibers, beating the stock, screening the

stock and introducing raw sulphite into the stock, introducing bleach into the stock, such as bleaching chlorine and passing the stock through a succession of bleaching towers.

65 9. In a process of manufacturing paper from refuse paper stock having relatively short fibers, beating the stock, screening the stock and introducing raw sulphite into the stock, such as bleaching chlorine, stirring said stock and bleaching with the raw sulphite and passing the stock successively from the top to the bottom of bleaching towers. 70

75 10. In the process of manufacturing paper from refuse stock, beating the refuse stock, cooking it to de-ink it, introducing surplus liquor from previous stock, extracting foreign material from the stock, screening it, introducing bleach into it and introducing raw sulphite into it. 80

85 11. In a process of manufacturing paper from refuse stock, beating the refuse stock, cooking it to de-ink it, introducing surplus liquor from previous stock, extracting foreign material from the stock, screening it, introducing bleach into it and introducing raw sulphite into it, and stirring it with 90 raw sulphite. 90

95 12. In a process of manufacturing paper from refuse stock, beating the refuse stock, cooking it to de-ink it, introducing surplus liquor from previous stock, extracting foreign material from the stock, screening it, introducing bleach into it, introducing raw sulphite into it, stirring it with the bleach 100 and the raw sulphite, and grinding the raw sulphite prior to its introduction. 100

105 13. In a process of manufacturing paper stock from refuse paper, beating the refuse paper into a paper stock having relatively short fibers, beating raw sulphite having relatively long fibers, introducing said beaten products one into the other, and introducing bleach into the combination. 110

In testimony whereof, I affix my signature. 115

HERBERT W. SERVER.

115

120

125

130